

## UNITED STATES PATENT OFFICE

2,061,897

## CORROSION-RESISTANT TUBE

Donald K. Crampton, Marion, and Newell W. Mitchell, Waterbury, Conn., assignors to The Chase Companies, Incorporated, Waterbury, Conn., a corporation of Connecticut

No Drawing. Application June 25, 1936.  
Serial No. 87,218

8 Claims. (Cl. 138—47)

This invention relates to improvements in corrosion-resistant tubes, and more particularly, corrosion-resistant wrought-metal tubes formed of copper-base alloys containing copper, nickel, aluminum and tin, with or without other ingredients which do not seriously impair the properties of the alloy.

This application is a continuation-in-part of our application Serial No. 709,172, filed January 31, 1934.

One object of this invention is to provide a tube formed of a copper-base alloy having superior resistance to corrosion.

Another object is to provide a tube formed of a copper-base alloy having superior resistance to corrosion and superior physical properties.

A further object is to provide a tube formed of a copper-base alloy having superior resistance to corrosion with capacity for being readily hot worked.

A still further object is to provide a tube formed of a copper-base alloy having both superior resistance to corrosion and capacity for being conveniently cold worked.

Another object is to provide a tube formed of a corrosion-resistant copper-base alloy which may be conveniently worked, either hot or cold.

Other objects and advantages will appear to those skilled in the art from the following, considered in conjunction with the appended claims.

In order that the pertinence of the following may be better understood, it may here be stated that binary alloys of copper-nickel, copper-aluminum, and copper-tin are well known in the art, as are also ternary alloys of copper-nickel-aluminum, copper-nickel-tin, and copper-aluminum-tin.

The present invention contemplates wrought-metal, corrosive-fluid-contact tubes, pipes and the like, such for example, as condenser and heat-exchanger tubes formed of a copper-base alloy in which, in addition to a preponderant amount of copper, nickel, aluminum and tin are included in suitable amounts, substantially without in the limits,—nickel about 4% to about 30%, aluminum about  $\frac{1}{2}$ % to about 4%, tin about  $\frac{1}{2}$ % to about 5%, and copper comprising substantially the remainder, that is, with or without other ingredients which do not seriously impair the properties of the alloy,—whereby improved corrosion-resistant characteristics are secured, together with other advantages.

*Tensile strength, ductility, etc.*

A series of studies of alloys within the ranges above set forth show, for example, that an alloy composed of about 5% nickel, 1% aluminum, 3% tin and a balance substantially all copper, possessed appreciably better physical properties than one containing about 5% nickel, 1% aluminum,

no tin, and the balance copper. The inclusion of the 3% of tin not only raised the tensile strength of the material in the worked and annealed state from approximately 43,400 lbs. per square inch to 57,300 lbs. per square inch, but 5 did so without any loss of ductility; the elongation in two inches being 34% for both of the alloys just referred to. The foregoing clearly shows that the inclusion of the tin added to the tensile strength in an amount approximately 10 13,900 lbs. per square inch without, however, harmfully affecting the ductility.

Further studies showed that an alloy containing about 5% nickel, 3% aluminum, 3% tin and the balance copper, possessed a tensile strength 15 about 69,400 lbs. per square inch and an elongation in two inches of 42%, whereas an alloy of about 5% nickel, 3% aluminum, no tin and the balance substantially all copper, possessed a tensile strength of but 58,000 lbs. per square inch 20 and an elongation in two inches of 28%. Thus it appears that the inclusion of 3% tin in the alloy just referred to increased the tensile strength some 11,400 lbs. per square inch, and at the same time accomplished what is unusual, 25 namely, an increase in elongation of some 14%. Usually, changes in alloys which produce increased tensile strength will result in a corresponding decrease in elongation.

Generally speaking, tests which have been conducted indicate that an increased nickel content has relatively little effect on the hot-working properties of the alloy but serves to gradually increase the hardness and toughness and, by the same token, increases the resistance to 35 cold-working. With increasing aluminum content, the hot workability seems to be appreciably improved, but the cold-workability is, on the contrary, somewhat decreased. In general the higher the nickel and/or aluminum content, a 40 relatively-lesser amount of tin is desirable in order to still preserve a commercially-workable product. From the standpoint of workability—both hot and cold—alloys containing from about 5% to about 10% nickel, from about 1% to 45 about 3% aluminum, and from about 1% to about 3% tin, have proved to be extremely satisfactory. Greater corrosion-resistance may be obtained, however, by raising the tin content up 50 toward the 5% mark, but with some loss in workability.

The properties above referred to were apparent when the material was in the annealed condition, but tests have also shown that the advantages of the tin content were also apparent when the material was in the age-hardened condition. Most of the alloys herein referred to possess to a greater or lesser degree, capacity for being age-hardened.

## Corrosion—resistance

A series of corrosion tests of the water-line type enduring for about one hundred days in dilute synthetic sea water at a temperature of 60° C. served to clearly demonstrate the possibility of securing superior all-around corrosion-resistance by the inclusion of tin with nickel, aluminum and copper. The synthetic sea-water solution referred to has been previously found to be quite corrosive to copper-base alloys, as well as to other alloys, and represents, moreover, a condition which is very commonly encountered in commercial practice, such, for instance, as in harbors. The synthetic sea water employed in the tests now being referred to was of a concentration about one-sixth that of full strength sea water, and has been found from extensive tests to be in general more corrosive than normal sea water itself.

The results obtained from the corrosion tests above referred to are given below in terms of per cent loss of original tensile strength, and for purposes of comparison straight copper-nickel-aluminum alloys are included, as well as so-called "Admiralty" brass, which latter alloy has heretofore been very largely used in condenser tubes, etc., subjected to corrosive waters:

| 30    | Composition of alloy |    |    |    |    | Percent of original strength lost by corrosion |
|-------|----------------------|----|----|----|----|------------------------------------------------|
|       | Cu                   | Ni | Al | Sn | Zn |                                                |
| No. 1 | 94                   | 5  | 1  |    |    | 13                                             |
| No. 2 | 91                   | 5  | 1  | 3  |    | 8                                              |
| No. 3 | 92                   | 5  | 3  |    |    | 3                                              |
| No. 4 | 89                   | 5  | 3  | 3  |    | 1                                              |
| No. 5 | 70                   |    |    | 1  | 29 | 42                                             |

The foregoing table shows that all of the copper-nickel-aluminum alloys, as well as the copper-nickel-aluminum-tin alloys of the present invention, are markedly superior to the "Admiralty" brass (#5). What is most pertinent, however, the results tabulated clearly show the superior corrosion-resistance of the quaternary alloy of the present invention over that of the ternary copper-nickel-aluminum alloys. The corrosion-test results further show that under the conditions referred to, the quaternary alloys of the present invention, with a 5% nickel content, are more resistant to corrosion with 3% aluminum than they are with but 1% aluminum.

Further corrosion tests in two other corrosive solutions confirm the corrosion-test results above given, as will be clear from the following table:

| 60     | Composition of alloy |    |    |    | Percent loss of original tensile strength in 2% malic acid and 2% sodium chloride solution; 50 day exposure (water line) 60° C. | Percent of loss of original tensile strength in 1% sulphuric acid solution; 10 day exposure (water line) 30° C. |
|--------|----------------------|----|----|----|---------------------------------------------------------------------------------------------------------------------------------|-----------------------------------------------------------------------------------------------------------------|
|        | Cu                   | Ni | Al | Sn |                                                                                                                                 |                                                                                                                 |
| No. 6  | 94                   | 5  | 1  |    | 21                                                                                                                              | 28                                                                                                              |
| No. 7  | 93                   | 5  | 1  | 1  | 17                                                                                                                              | 17                                                                                                              |
| No. 8  | 91                   | 5  | 1  | 3  | 10                                                                                                                              | 14                                                                                                              |
| No. 9  | 92                   | 5  | 3  |    | 17                                                                                                                              | 29                                                                                                              |
| No. 10 | 91                   | 5  | 3  | 1  | 16                                                                                                                              | 14                                                                                                              |
| No. 11 | 89                   | 5  | 3  | 3  | 12                                                                                                                              | 9                                                                                                               |
| No. 12 | 89                   | 10 | 1  |    | 15                                                                                                                              | 23                                                                                                              |
| No. 13 | 88                   | 10 | 1  | 1  | 13                                                                                                                              | 18                                                                                                              |

The alloys referred to in the preceding table were all heat-treated for about one and one-half hours at a temperature of 600° C. to build up a considerable surface-film with the intent

of taking advantage as much as possible of the film-forming characteristic of the aluminum constituent.

The results of the foregoing tests in general confirm the findings from the previous corrosion tests hereinbefore tabulated, and indicate that the effect of the larger aluminum content is not, however, here so marked as in the previous test referred to, but the beneficial effect of larger tin content is very marked.

The combined malic acid and sodium chloride solution referred to is comparable in its general effect to many corrosive food stuffs, and it has been found to have a very powerful corrosive effect on a wide variety of alloys. The 1% sulphuric acid solution referred to is representative of a relatively-strong acid-condition—a condition quite commonly found in practice—and very corrosive to a wide variety of alloys.

A further series of corrosion tests employing a markedly strong acid solution (5% H<sub>2</sub>SO<sub>4</sub>) is clearly indicative of the superior corrosion-resistant properties of alloys of the present invention, as set forth in the following table. The alloys when subjected to the tests were in the annealed state.

|        | Composition of Alloy |    |     |    |    |    | Per cent loss of original tensile strength in 5% sulphuric acid solution; 6 day exposure (water line) 30° C. |
|--------|----------------------|----|-----|----|----|----|--------------------------------------------------------------------------------------------------------------|
|        | Cu                   | Ni | Al  | Sn | Mn | Zn |                                                                                                              |
| No. 14 | 93.5                 | 5  | 1.5 |    |    |    | 18                                                                                                           |
| No. 15 | 90.5                 | 5  | 1.5 | 3  |    |    | 3                                                                                                            |
| No. 16 | 88.5                 | 5  | 1.5 | 5  |    |    | 5                                                                                                            |
| No. 17 | 85.5                 | 10 | 1.5 | 3  |    |    | 2                                                                                                            |
| No. 18 | 83.5                 | 10 | 1.5 | 5  | 1  |    | 5                                                                                                            |
| No. 19 | 89.5                 | 5  | 1.5 | 3  |    |    | 7                                                                                                            |
| No. 20 | 89.5                 | 5  | 1.5 | 3  | 1  |    | 6                                                                                                            |
| No. 21 | 84.5                 | 10 | 1.5 | 3  | 1  |    | 40                                                                                                           |
| No. 22 | 84.5                 | 10 | 1.5 | 3  | 1  |    | 16                                                                                                           |
| No. 23 | 100                  |    |     |    |    |    |                                                                                                              |

Alloys Nos. 19, 20, 21 and 22 serve to show that the inclusion of manganese or zinc does not detract from the corrosion-resistance of the alloys under the conditions given. On the other hand, it may be stated that manganese serves as an excellent deoxidizer for such nickel-bearing alloys and the zinc serves to facilitate the making of sound castings.

As hereinbefore pointed out, the present invention contemplates a copper-nickel-aluminum-tin alloy comprising essentially nickel about 4% to about 30%, aluminum about 1/2% to about 4%, tin about 1/2% to about 5%, and a balance substantially all copper, save that allowance should be made for miscellaneous ingredients present either as impurities or intentionally incorporated if desired.

The following represent a few specific alloys coming within the scope of the present invention in addition to those hereinbefore given and are to be considered in all respects as representative and not exhaustive:

| Cu   | Ni | Al  | Sn | Si | Fe  | Mn  | Zn  | P  | Od |
|------|----|-----|----|----|-----|-----|-----|----|----|
| 68   | 30 | 1   | 1  |    |     |     |     |    |    |
| 77   | 20 | 2   | 1  |    |     |     |     |    |    |
| 86.6 | 10 | 2   | 1  |    |     |     |     |    |    |
| 87   | 5  | 3   | 3  |    | .5  | .5  | 1.0 | .4 |    |
| 87   | 4  | 4   | 4  | .1 | .25 | .15 | .5  |    |    |
| 85   | 10 | 1.5 | 3  |    |     |     |     |    | .5 |

The invention may be carried out in other specific ways than those herein set forth without

departing from the spirit and essential characteristics of the invention, and the present embodiments are therefore to be considered in all respects as illustrative and not restrictive, and all changes coming within the meaning and equivalency range of the appended claims are intended to be embraced therein.

We claim:

1. A corrosion-resistant wrought-metal tube formed from an alloy containing: about 4% to about 30% nickel; about  $\frac{1}{2}\%$  to about 4% aluminum; about  $\frac{1}{2}\%$  to about 5% tin; and the balance substantially of copper.
2. A corrosion-resistant wrought-metal tube formed from an alloy containing: about 4% to about 20% nickel; about  $\frac{1}{2}\%$  to about 4% aluminum; about  $\frac{1}{2}\%$  to about 5% tin; and the balance substantially of copper.
3. A corrosion-resistant wrought-metal tube formed from an alloy containing: about 4% to about 15% nickel; about  $\frac{1}{2}\%$  to about 4% aluminum; about  $\frac{1}{2}\%$  to about 5% tin; and the balance substantially of copper.
4. A corrosion-resistant wrought-metal tube

formed from an alloy containing: about 4% to about 10% nickel; about  $\frac{1}{2}\%$  to about 4% aluminum; about  $\frac{1}{2}\%$  to about 5% tin; and the balance substantially of copper.

5. A corrosion-resistant wrought-metal tube formed from an alloy containing: about 5% to about 10% nickel; about 1% to about 3% aluminum; about 1% to about 3% tin; and the balance substantially of copper.

6. A corrosion-resistant wrought-metal tube formed from an alloy containing: about 20% nickel; about 2% aluminum; about 1% tin; and the balance substantially of copper.

7. A corrosion-resistant wrought-metal tube formed from an alloy containing: about 10% nickel; about 3% aluminum; about 3% tin; and the balance substantially of copper.

8. A corrosion-resistant wrought-metal tube formed from an alloy containing: about 5% nickel; about 3% aluminum; about 3% tin; and the balance substantially of copper.

DONALD K. CRAMPTON.  
NEWELL W. MITCHELL.